# EUROPEAN PATENT SPECIFICATION

(11) **EP 1 907 198 B1**
(45) Date of publication and mention of the grant of the patent: **11.08.2021**
(21) Application number: 05756917.0
(22) Date of filing: 29.06.2005
(51) Int. Cl.: B31F 1/07

(54) **PROCESS FOR SOFTENING HYGIENIC PAPER**
VERFAHREN ZUM WEICHMACHEN VON HYGIENEPAPIER
PROCEDE D'ADOUCISSEMENT DE PAPIER HYGIENIQUE

(43) Date of publication of application: 09.04.2008
(73) Proprietor: Henkel AG & Co. KGaA, 40589 Düsseldorf (DE)
(72) Inventor: CARRARA, Stefano, I-24044 Dalmine (IT); GRANELLI, Marco, I-24126 Bergamo (IT); CAVALLI, Dario, I-20125 Milano (IT)
(86) International application number: PCT/EP2005/006960
(87) International publication number: WO 2007/000177

(56) References cited:
- EP-A- 1 233 107
- WO-A-00/04230
- WO-A-99/59808
- WO-A1-2006/071147
- DE-A1- 19 732 735
- US-A- 4 135 024
- US-A- 4 481 243
- US-A1- 2003 041 989
- US-A1- 2004 168 780
- US-B1- 6 551 691
- US-B1- 6 602 387

## Description

The invention relates to a process for producing multi-layer hygiene paper and hygiene tissues from various generally web-shaped starting materials forming the individual layers of the finished products, whereby the starting materials are supplied from material supply stations and continuously processed whereby an additional process step for an application of a softening composition to such multi-layer paper is included in the process. The invention relates also to the multi-layer products manufactured by such process.

Methods and apparatus for the manufacture of multi-ply tissues and papers are known in the art and are used for producing facial tissues, bath tissues, hygiene pads, liners, hygiene paper and the like. Such modern hygiene products of this type generally comprise several layers that are connected together in a sandwiched or multi-ply structure. For this purpose, it is typical to supply narrow webs or bands of various starting materials from large supply rolls to the actual processing stations in which the starting materials are processed in a suitable manner to form the finished products.

Such hygiene products are frequently applied and come into contact with the skin. During frequent use, the skin may be compromised and can become so abraded that it might become red and sore to the touch. Additionally, the feeling of the surface may be hard and stiff but it should provide a soft feeling. In order to address these concerns, there have been numerous previous attempts to reduce the abrasive effect of such tissues and to increase their softness. One common approach to increase the softness of hygiene products is by closely controlling the mechanical processing of the paper web. By using particular processing steps during papermaking such paper or tissue products can be made that are softer and less irritating. Besides mechanical processing, other patents describe the use of emollients, lubricants and cleansing agents and the like to such products to enhance the softness impression and to reduce irritation on the skin. To add such wet additives during the paper making process raise the problem of wet strength stability of the web.

US 2003/0059579 describes a sanitary paper tissue product consisting of several plies. On the outer surfaces a chemical softening composition out of polysiloxan-polyalkyleneoxide copolymer is applied. This application is performed during the paper making process that means after the web has been prepared and dried and is still warm from this process the softening solution is applied and thereafter the web is wound on rolls.

WO 03/027390 describes a soft tissue paper product which comprises on the outer surface of that tissue a chemical softening composition comprising a polysiloxan-copolymer. This softening agent is applied during the web making process after the web has been dried and thereafter this web is wound on rolls.

US 6,551,691 describes an absorbent paper product consisting out of several plies. These plies are glued together and are subjected to an embossing step. The embossed plies may contain a softening agent but no specific description of this softening agent is made.

This prior art always includes the application of the softening agent in the web making process either to the wet web or to the dry web. Thereafter the rolls of web are stored and transported to the tissue making companies and at that stage the different layers are bound together and the multi-ply product is made. It is a disadvantage that already during the paper making process the different softeners need to be applied. So on a later stage in the plant making the multi-ply products no change or adaptation to a different softening agent is possible. So the process is less flexible. Additionally during rolling and transport of the paper rolls the soft surface is frequently damaged and the later manufactured products do not show adequate surface softness as provided originally to the single web after manufacture.

US 6,602,387 B1 discloses paper tissues comprising at least two plies and having a specific physiological surface smoothness. A preferred process to obtain a respective ply comprises a step of applying lotion preferably to the surfaces constituting the outermost multi-ply tissue surfaces, and a step of attaching the individual plies by embossing. Optionally, an additional step of applying glue, preferably only to the raised portions of the textured plies, may be performed.

DE 19732735 A1 discloses methods for the manufacturing of multi-ply tissue products, comprising the steps of providing a plurality of webs; adjoining said webs so as to obtain an untreated multi-ply paper product, wherein the adjoining and ply-bonding is realized by means of embossing; and applying a softening composition to both outer surfaces of said multi-ply paper product so as to obtain a multi-ply tissue product treated with a softening composition. The softening composition used comprises a quaternary ammonium compound in an amount of from 3 to 30 wt.-%, a siloxane foam inhibitor in an amount of from 0.1 to 3.0 wt.-%, aloe vera powder in an amount of from 0.01 to 10 wt.-%, a polyhydroxy plasticizer in an amount of from 0.05 to 5 wt.-%, and water in an amount of from about 52 to 97 wt.-%.

The present invention therefore provides a process to manufacture multi-ply paper products whereby during the manufacture and preparation of a web as precursor material no addition of a softening composition or a softening step is required. The soft feel character shall be applied to the ready made product during the processing step of manufacturing the multi-ply paper product out of the single webs. The scope of protection in defined by the appended claims.

The problem is solved by a process for manufacturing a multi-ply hygiene paper product according to the features of independent claim 1. The process for manufacturing a multi-ply hygiene paper product comprising supplying at least two separate web materials to a processing station, applying to at least one of the surfaces of the webs forming an outer ply a softening composition, adjoining the web layers by glueing and/or embossing to manufacture a multi-ply hygiene paper and transporting such product to a cutting and/ or further processing station.

The substrates for manufacturing multi-ply paper products are known. They consist of webs of different size. The single webs to be adjoined may consist of various natural fibers preferably from wood pulp but other cellulosic fibrous pulp fibers such as cotton, linters, bagasse, etc. can be utilized. Also synthetic fibers may be used such as polyethelene, polypropylene or polyamide fibers, also a combination of synthetic and natural fibers is possible. The obtained product shall form a paper or tissue web.

The present invention is useful with tissue paper and hygiene paper in general, such paper or tissue products according to the invention are always multi-ply materials of at least two webs. The webs may consist of conventionally pressed paper, densified paper or uncompacted paper. During the paper making process various chemicals may be added to the fiber materials, e.g. for improving wet strength, lubricants and other common additives to be selected according to the specific use of the product. Such additives applied during the paper making or web making process are known in the prior art. After the web is completed and dried it is wound to rolls which may be stored.

An apparatus for manufacturing multi-ply paper products is generally known. It comprises a plurality of processing stations as well as a plurality of supply stations. The supply stations feed web-shaped starting materials, which shall form the individual layers and parts of the finished paper product. The starting material is stored on supply rolls which are transported from the supply stations to the processing stations where the different webs are processed to form the finished multi-ply product.

More particularly, the processing stations may include printing stations, embossing and/or stamping stations as well as a cutting station for respectively embossing or stamping and cutting the material in the process of manufacturing the paper product. Additionally, at least one adhesive applicator device for applying glue or other adhesives onto the webs forming the multi-ply products is present. The apparatus further includes transport arrangements for transporting on-line the materials through the processing stations, including web guidance arrangement for guiding the web among the respective processing stations. According to the invention at least one applicator device for the application of a softener composition is included, which shall coat at least one surface with a softener composition.

The web-shaped starting material is initially supplied and stored in a condition rolled-up on supply rolls in the supply stations. From there, the web-shaped starting material runs from the supply rolls through a material web store, which may have any conventional construction and operation. The process according to the invention shall proceed continuously, so a respective web end splicer device may be arranged after the supply roll.

According to the process the different webs used in the multi-ply product may be identical or may consist of different materials.

An apparatus to be utilised according to the process shall include suitable transport and guide arrangements so that the web-shaped starting material can be rolled from the supply roll and then driven and deflected as necessary to be supplied from the supply roll to the processing stations.

Optionally as first processing station a printing station can be integrated in the apparatus. The web which shall constitute the outer surface of the multi-ply product may be printed. Such printing stations are known and can be easily integrated in this process. Only one printing station for one surface may be integrated but it is also possible to imprint both outer layers of the product. As the printing ink many influence the surface of the web, this process step shall be performed prior to any softening step.

After the printing step and optionally after embossing the web but prior to the embossing station a softening composition is applied to at least one web of the multi-ply product. Such softening compositions are liquid products which may be applied by known devices to a web. This application may be performed by rolls, printing devices, nozzles or spray application. This can be performed to one web or in a parallel process step to two webs of the multi-ply product. The at least one web to be treated shall constitute an outer layer of the multi-ply product. The surface of the web to be treated with the softening composition shall constitute the outer surface of the finished multi-ply paper product. It is required for the process according to the invention that at least one outer surface shall show the soft feel effect. In one embodiment of the invention only to one of the outer web layers a softening agent is applied, another embodiment includes the application of such softening composition to both of the outer web layers.

The softener composition shall provide to the outer layers of the tissue or hygiene paper a soft feel effect. The amount of the softening composition applied in this process is between 1 to 10 g/m² preferably 2 to 7 g/ m² of the surface (wet composition).

Such application of a softening composition may be performed on different steps of the process due to the parallel processing of the webs to be adjoined. If only one outer web is subject to an embossing step the application of the softening composition may be performed directly after such embossing step. In such case it is possible not to coat the complete surface of the web with a softening composition, but only the upper parts of the embossed surface. In another embodiment of the invention the softener composition is applied directly after the printing step to one or more webs prior to adjoining the webs. In another embodiment of the invention the softening composition is applied to an outer web and to a different web an adhesive or glue is applied. Subsequently as next step of each process the different webs are adjoined together. In each case the softening composition according to the invention shall be composed of a waterborne material. It is not required to add a drying step before further processing the web. The additional moisture to be applied to the paper may be absorbed and distributed in the web without deteriorating the mechanical properties of the webs.

After application of the softening composition to at least one web the different webs shall be adjoined. This is performed by a combination of gluing and embossing the different webs together. For example as next step in the manufacturing process the webs may be subjected to an embossing step.

Conventional rotary embossing stations may be used to emboss the webs. Typical embossing stations may included rotary embossing rolls and cooperating, rotary anvil rolls. The embossing rolls have been configured to provide an array of embossing dies to provide embossing lines arranged with selected shapes. Other conventional embossing stations have also included bonding components for providing construction bonds. In particular systems, the construction bonds have been located proximate the regions of the web where the web has been embossed. Typically, the operating speed of the embossing system will be limited by the available embossing force and by the amount of dwell time needed to reliably form the desired embossments. The embossing operation is performed prior to a cutting operation that separates the multi-layer web into individual articles.

The embossing shall be accomplished while substantially avoiding undesired breaks or fractures of component portions of the web. It is known to add friction-reducing material to the web or a debonding agent. This may not be necessary when applying the softening composition prior to the embossing step, or the softening composition may include such ingredients. The moisture content of the cellulosic fibers shall be controlled during the embossing process to support the embossing process without any interruption of the continuous process. To adjust a suitable moisture content the amount of the softening composition to be applied or water content may be adjusted.

After the application of the softening composition an additional process step for the application of a glue or an adhesive to the different webs is included in the process. Such adhesive shall provide a good adhesion between the different layers of the multi-ply product. Material and devices for the application of a glue or an adhesive to paper webs are already known. The adhesive is applied only to each second layer of the product. It is possible to apply such adhesive to the outer layer of the multi-layer product or preferably it may be applied to the layer adjacent to the outer layer of the multi-ply product. It is required not to apply the adhesive to the surface which has already been coated with the softening composition and if possible to select a different web.

The adhesives may be applied over the whole surface of the web, in a variety of patterns on a surfaces, connecting at least portions of the adjacent surface of one layer with portions of the adjacent surface of the next layer, or it may be applied in form of signs, logos, letters and the like to a surface. In such case the adhesive may be coloured.

Any operative adhesive applicator may be employed. Suitable applicators can include adhesive spray devices, adhesive coating devices, adhesive printing devices, or the like, as well as combinations thereof. Any operative adhesive may be employed. For example suitable adhesives can include hot melt adhesives, pressure-sensitive adhesives, solvent-based adhesives or waterborne adhesives. Preferably such adhesives are hot melt adhesives. Such hot melt adhesives can contain polymers based on polyesters, polyuretanes, polyamides, polyacrylates or polyolefines. Another embodiment of the invention applies waterborne adhesives to the webs. Examples of such adhesives are described in EP 1085973. The adhesive may contain dyes or pigments, so that its printing patterns may be visible and may serve as printing step. The adhesives may be applied to the surface as continuous film or in a certain pattern. Additionally it is possible to apply the coating only on the upper part of an embossed web so that only such upper parts are glued to the adjacent web surface. Such application technology and the respective devices for the application are generally known.

According to the invention to improve the soft feel effect of the multi-ply paper a softening composition has to be applied to at least one outer surface of the multi-ply paper. Such softening compositions are already known. A waterborne softening composition is used in a process according to this invention. Such softening composition shall include a softening agent, water and other useful ingredients like conditioners, surfactants, organic solvents, builders, bleaching agents, complexing agents, perfumes, dyes, biological active compounds, stabilizers and other components. The softening compositions used for the present invention may additionally comprise lubricants, a structurant or rheology enhancer like thickeners.

As softening agent most preferably quaternary ammonium compounds, cationic polymers or cationic surfactants are preferred. Quaternary ammonium compounds are commonly known under the name of esterquat. Cationic polymers may include for example polyquaternary polymers like grafted cellulose derivates, cationic cellulose derivates, cationic quaternary sugar derivates and/or amino silicon copolymers.

Other non-ionic softening agents may be included in the composition additionally. Examples of such components are polyoxyalkylene-glycerolalcanoate, polybutylene, long chain fatty acids, ethoxylated fatty acidamides, alcylpolyglycosides or fatty acid esters of polycarboxylic acids. The softening composition may contain one or more of such softening components. It shall be include in an amount of 3 to 35 % by weight of the total composition.

In order to enhance the application process and the properties of the multi-ply product, additional ingredients can be incorporated into the softener composition. The classes of ingredients and their corresponding benefits include, without limitation: antifoaming agents; preservatives; antimicrobial actives, antiseptic actives; antioxidants; astringents , biological additives, vitamins, botanical extracts, proteins, peptides, skin protectants, lipids, sterols; colorants ; deodorants, fragrances ; moisturizers, humectants; lubricants, such as silicones and organomodified silicones; skin protectants, UV absorbers, optical brighteners and waxes.

Another class of additives are components for regulating the viscosity, e. g. thickeners. Such additives include inorganic or organic components like natural polymers , like xanthane, agar-agar, cellulosic polymers or synthetic polymers, like (meth)acrylicacids, or silicates, like bentonite, montmorillonite, aluminium silicate. In combination with the solvents it is possible to adjust the viscosity of the softening composition according to the requirements of the application device. Additionally, a hydrophilic surfactant may be utilized to emulsify various ingredients into the formulation, and improve wettability of the product. Such additives shall be present in an amount from 0,1 to 10 % of the composition.

A softening composition suitable for the invention contains water. The amount of water may range between 20 % to 90 %, preferably between 40 % to 80 %. It may include additionally organic solvents in particular low molecular alcohols. Such alcohols include liquid polyethylenglycols with low molecular weight e. g. with a molecular weight of 200 to 600 g/mol. Other useful solvents are alcohols like ethanol, isopropanol, n-propanol; ketones like aceton and methylethylketone; C₂ to C₆ polyols in particular dioles or trioles like ethyleneglycol, propyleneglycol, glycerin or mixtures thereof. The organic solvents may be included in an amount between 0,1 % to 30 % in particular from 3 % to 15 %.

Waterborne softening compositions which may be used in the process of the invention are for example described in DE 10339761 or EP 1097270.

The application of the softening composition may be performed by known methods.

Such methods include, for example, spraying, printing, coating, extrusion, ink jet printing, and combinations thereof. It should be applied in such a manner that the tissue does not become oversaturated with the softening formulation. If oversaturation occurs this may lead to a substantial decrease in the tensile strength of the web and poor aesthetic performance. After application of the softening composition the web shall not contain too much humidity in order not to deteriorate the strength of the web during processing. When applied to the paper product, the softening compositions described herein shall impart a soft feel to the touch.

According to one embodiment of the invention the paper webs constituting the outer layers are printed, coated with a softening composition, embossed and glued to other webs composing the other layers of the product. After the multi-ply product is formed the product is conveyed to a cutting station. Such cutting stations are generally known. They manufacture out of the web shaped multi-ply product the ready made form. This may include rolls of paper, folded paper, and the like. During each process step after the application of the softening composition the handling of the web shall be arranged to avoid additional strong pressing steps to the outer surface of such multi-ply product.

Another embodiment of the invention consists of a multi-ply paper or tissue product manufactured according to the process of this invention. It consists of at least two layers of paper or similar fibrous sheets, which at least on one outer side of the surface show a soft feel effect. It may also contain several layers, preferably 3 to 5, which may consist of the same material or of different materials, having different mechanical performance. The multi-ply paper may show one imprinted and/or embossed outer surface but it is also possible to have two imprinted and/or embossed surfaces. The product shall be manufactured according to the process of the invention. The softening composition shall not be incorporated during the paper making process but shall be applied on-line during the adjoining step of the different layers.

The multi-ply product manufactured in a process according to the invention shows on at least one surface a soft feel effect. Such effect will be maintained during the preparation of the ready made product. The absorbed softening composition does not significantly deteriorate the embossing step and the gluing step that means the further processing of the single webs in the process is not impaired. Especially the speed of manufacture of the processing line is similar to the processing speed without the application step of the softening agent. So according to the invention a multi-ply product in form of paper or tissue product is manufactured by a process which shows an improved flexibility in the manufacture by changing the softening composition in the process so that different types of multi-ply paper may be manufactured. Additionally according to the process of the invention the number of steps which may disturb the soft feel surface of the web is reduced as the softening agent may be applied at a very late production stage.

## Claims

1. A process for manufacturing a multi-ply hygiene paper product comprising
a) supplying at least two separate webs to a processing station,
b) applying to at least one of the surfaces of at least one of the webs forming an outer ply a softening composition, wherein the softening composition is applied to at least one of the outer surface of the multi-ply hygiene paper product,
c) applying to at least one web an adhesive layer, wherein the adhesive layer is applied to the surface which is not coated with the softening composition,
d) adjoining the webs by embossing to manufacture a multi-ply hygiene paper
e) transporting such paper to a cutting and/ or further processing station,
wherein the softening composition is a waterborne solution which comprises from 20 to 90 wt.% of water and wherein the different webs are adjoined after application of the softening composition to the at least one web,
wherein steps a)-e) are carried out in a consecutive order.

2. A process according to claim 1, wherein the softening composition is applied to both outer webs.

3. A process according to claim 1 or 2, wherein the softening composition is applied to both outer surfaces of the multi-ply product.

4. A process according to any one of claims 1 to 3, wherein the softening composition is applied by means for printing, spraying or rolling.

5. A process according to any one of claims 1 to 4, wherein a waterborne adhesive or a hot melt adhesive is applied.

6. A process according to any one of claims 1 to 5, wherein adhesive layers are applied in a manner so that every two adjacent layers are bonded by one adhesive layer.

7. A process according to any one of claims 1 to 6, wherein a printing step is applied to the web prior to the application of the softening composition or after such application of softening composition.

8. A process according to any one of claims 1 to 7, wherein no supplemental drying step is performed on such web after the application of the softening composition.

9. A process according to any one of claims 1 to 7, wherein an additional drying step is applied subsequent to the application of the softening composition.

10. A process according to any one of claims 1 to 9, wherein the softening composition is applied between 1 to 10 g/m² on each surface, preferably between 2 to 7 g/m².

11. A process according to any one of claims 1 to 10, wherein the softening composition contains 3 % to 35 % by weight of one or more softening agents, preferably at least one esterquat, 0,1% to 30 % by weight of low molecular weight alcohols, and 0,1% to 10 % by weight of additives.

12. A multi-ply hygiene paper manufactured according to any one of claims 1 to 11, comprising at least two plies wherein to at least one of the outer plies a waterborne softening composition was applied during manufacturing such multi-ply paper out of the webs, wherein to at least one of the outer surfaces of the outer ply said waterborne softening composition was applied.

13. A multi-ply hygiene paper according to claim 12, wherein to the outer surfaces of both outer plies a waterborne softening composition was applied.

14. A multi-ply hygiene paper according to claim 12 or 13, consisting of at least three plies.

15. A multi-ply hygiene paper according to any one of claims 12 to 14, wherein the softening composition is applied between 1 to 10 g/m² on the respective surface.

16. A multi-ply hygiene paper according to any one of claims 12 to 15, wherein the softening composition contains 3 % to 35 % by weight of one or more softening agents, preferably at least one esterquat, 0,1% to 30 % by weight of low molecular weight alcohols, and 0,1% to 10 % by weight of additives.

17. A multi-ply hygiene paper according to any one of claims 12 to 16, wherein a waterborne adhesive or a hotmelt adhesive is used.

## Patentansprüche

1. Vorgang zum Herstellen eines mehrlagigen Hygienepapierprodukts, umfassend
a) Zuführen von mindestens zwei getrennten Bahnen zu einer Verarbeitungsstation,
b) Auftragen, auf mindestens eine der Oberflächen von mindestens einer der Bahnen, die eine äußere Lage ausbilden, einer weichmachenden Zusammensetzung, wobei die weichmachende Zusammensetzung auf mindestens eine der äußeren Oberflächen des mehrlagigen Hygienepapierprodukts aufgetragen wird,
c) Auftragen, auf mindestens eine Bahn, einer Klebstoffschicht, wobei die Klebstoffschicht auf die Oberfläche aufgebracht wird, die nicht mit der weichmachenden Zusammensetzung beschichtet ist,
d) Verbinden der Bahnen durch Prägen, um ein mehrlagiges Hygienepapier herzustellen
e) Transportieren dieses Papiers zu einer Schneide- und/oder Weiterverarbeitungsstation,
wobei die weichmachende Zusammensetzung eine wässrige Lösung ist, die von 20 bis 90 Gew.-% Wasser umfasst, und wobei die unterschiedlichen Bahnen nach der Auftragung der weichmachenden Zusammensetzung auf die mindestens eine Bahn verbunden werden,
wobei die Schritte a)-e) in einer aufeinanderfolgenden Reihenfolge ausgeführt werden.

2. Vorgang nach Anspruch 1, wobei die weichmachende Zusammensetzung auf beide äußeren Bahnen aufgetragen wird.

3. Vorgang nach Anspruch 1 oder 2, wobei die weichmachende Zusammensetzung auf beide äußere Oberflächen des mehrlagigen Produkts aufgetragen wird.

4. Vorgang nach einem der Ansprüche 1 bis 3, wobei die weichmachende Zusammensetzung durch Mittel zum Drucken, Sprühen oder Walzen aufgetragen wird.

5. Vorgang nach einem der Ansprüche 1 bis 4, wobei ein wässriger Klebstoff oder ein Heißschmelzklebstoff aufgetragen wird.

6. Vorgang nach einem der Ansprüche 1 bis 5, wobei Klebstoffschichten auf eine Weise aufgetragen werden, sodass jeweils zwei angrenzende Schichten durch eine Klebstoffschicht verklebt werden.

7. Vorgang nach einem der Ansprüche 1 bis 6, wobei ein Druckschritt auf die Bahn vor der Auftragung der weichmachenden Zusammensetzung oder nach einer solchen Auftragung der weichmachenden Zusammensetzung angewendet wird.

8. Vorgang nach einem der Ansprüche 1 bis 7, wobei nach der Auftragung der weichmachenden Zusammensetzung kein zusätzlicher Trocknungsschritt an einer solchen Bahn durchgeführt wird.

9. Vorgang nach einem der Ansprüche 1 bis 7, wobei anschließend an die Auftragung der weichmachenden Zusammensetzung ein zusätzlicher Trocknungsschritt angewendet wird.

10. Vorgang nach einem der Ansprüche 1 bis 9, wobei die weichmachende Zusammensetzung zwischen 1 bis 10 g/m² auf jede Oberfläche aufgetragen wird, vorzugsweise zwischen 2 bis 7 g/m².

11. Vorgang nach einem der Ansprüche 1 bis 10, wobei die weichmachende Zusammensetzung 3 bis 35 Gew.-% eines oder mehrerer Weichmacher, vorzugsweise mindestens ein Esterquat, 0,1 bis 30 Gew.-% Alkohole mit einem niedrigen Molekulargewicht und 0,1 bis 10 Gew.-% Zusätze enthält.

12. Mehrlagiges Hygienepapier, das nach einem der Ansprüche 1 bis 11 hergestellt wird, umfassend mindestens zwei Lagen, wobei auf mindestens eine der äußeren Lagen während der Herstellung eines solchen mehrlagigen Papiers aus den Bahnen eine wässrige weichmachende Zusammensetzung aufgetragen wurde, wobei auf mindestens eine der äußeren Oberflächen der äußeren Lage die wässrige weichmachende Zusammensetzung aufgetragen wird.

13. Mehrlagiges Hygienepapier nach Anspruch 12, wobei auf die äußeren Oberflächen beider äußeren Lagen eine wässrige weichmachende Zusammensetzung aufgetragen wird.

14. Mehrlagiges Hygienepapier nach Anspruch 12 oder 13, bestehend aus mindestens drei Lagen.

15. Mehrlagiges Hygienepapier nach einem der Ansprüche 12 bis 14, wobei die weichmachende Zusammensetzung zwischen 1 bis 10 g/m² auf die jeweilige Oberfläche aufgetragen wird.

16. Mehrlagiges Hygienepapier nach einem der Ansprüche 12 bis 15, wobei die weichmachende Zusammensetzung 3 bis 35 Gew.-% eines oder mehrerer Weichmacher, vorzugsweise mindestens ein Esterquat, 0,1 bis 30 Gew.-% Alkohole mit einem niedrigen Molekulargewicht und 0,1 bis 10 Gew.-% Zusätze enthält.

17. Mehrlagiges Hygienepapier nach einem der Ansprüche 12 bis 16, wobei ein wässriger Klebstoff oder ein Heißschmelzklebstoff verwendet wird.

## Revendications

1. Procédé de fabrication d'un produit en papier hygiénique à plusieurs épaisseurs comprenant
a) la fourniture d'au moins deux bandes distinctes à un poste de traitement,
b) l'application sur au moins une des surfaces d'au moins une des bandes formant une épaisseur externe d'une composition adoucissante, la composition adoucissante étant appliquée sur au moins une des surfaces externes du produit en papier hygiénique à plusieurs épaisseurs,
c) l'application sur au moins une bande d'une couche adhésive, la couche adhésive étant appliquée sur la surface qui n'est pas revêtue de la composition adoucissante,
d) la mise en contact des bandes par gaufrage pour fabriquer un papier hygiénique à plusieurs épaisseurs
e) le transport de ce papier jusqu'à un poste de découpe et/ou de traitement ultérieur,
dans lequel la composition adoucissante est une solution à base aqueuse qui comprend de 20 à 90 % en poids d'eau et dans lequel les différentes bandes sont mises en contact après application de la composition adoucissante sur l'au moins une bande,
dans lequel les étapes a) à e) sont exécutées dans un ordre consécutif.

2. Procédé selon la revendication 1, dans lequel la composition adoucissante est appliquée sur les deux bandes externes.

3. Procédé selon la revendication 1 ou 2, dans lequel la composition adoucissante est appliquée sur les deux surfaces externes du produit à plusieurs épaisseurs.

4. Procédé selon l'une quelconque des revendications 1 à 3, dans lequel la composition adoucissante est appliquée par des moyens d'impression, de pulvérisation ou de laminage.

5. Procédé selon l'une quelconque des revendications 1 à 4, dans lequel un adhésif à base aqueuse ou un adhésif thermofusible est appliqué.

6. Procédé selon l'une quelconque des revendications 1 à 5, dans lequel les couches adhésives sont appliquées de manière à ce que toutes les deux couches adjacentes soient liées par une couche adhésive.

7. Procédé selon l'une quelconque des revendications 1 à 6, dans lequel une étape d'impression est appliquée à la bande avant l'application de la composition adoucissante ou après une telle application de la composition adoucissante.

8. Procédé selon l'une quelconque des revendications 1 à 7, dans lequel aucune étape de séchage supplémentaire n'est effectuée sur cette bande après l'application de la composition adoucissante.

9. Procédé selon l'une quelconque des revendications 1 à 7, dans lequel une étape de séchage additionnelle est appliquée après l'application de la composition adoucissante.

10. Procédé selon l'une quelconque des revendications 1 à 9, dans lequel la composition adoucissante est appliquée entre 1 à 10 g/m² sur chaque surface, de préférence entre 2 à 7 g/m².

11. Procédé selon l'une quelconque des revendications 1 à 10, dans lequel la composition adoucissante contient 3 % à 35 % en poids d'un ou plusieurs agents adoucissants, de préférence au moins un esterquat, 0,1 % à 30 % en poids d'alcools de faible poids moléculaire, et 0,1 % à 10 % en poids d'additifs.

12. Papier hygiénique à plusieurs épaisseurs fabriqué selon l'une quelconque des revendications 1 à 11, comprenant au moins deux épaisseurs dans lequel une composition adoucissante à base aqueuse a été appliquée sur au moins une des épaisseurs externes pendant la fabrication de ce papier à plusieurs épaisseurs à partir des bandes, dans lequel ladite composition adoucissante à base aqueuse a été appliquée sur au moins l'une des surfaces externes de l'épaisseur externe.

13. Papier hygiénique à plusieurs épaisseurs selon la revendication 12, dans lequel une composition adoucissante à base aqueuse a été appliquée sur les surfaces externes des deux épaisseurs externes.

14. Papier hygiénique à plusieurs épaisseurs selon la revendication 12 ou 13, constitué d'au moins trois épaisseurs.

15. Papier hygiénique à plusieurs épaisseurs selon l'une quelconque des revendications 12 à 14, dans lequel la composition adoucissante est appliquée entre 1 et 10 g/m² sur la surface respective.

16. Papier hygiénique à plusieurs épaisseurs selon l'une quelconque des revendications 12 à 15, dans lequel la composition adoucissante contient 3 % à 35 % en poids d'un ou plusieurs agents adoucissants, de préférence au moins un esterquat, 0,1 % à 30 % en poids d'alcools de faible poids moléculaire et 0,1 % à 10 % en poids d'additifs.

17. Papier hygiénique à plusieurs épaisseurs selon l'une quelconque des revendications 12 à 16, dans lequel un adhésif à base aqueuse ou un adhésif thermofusible est utilisé.
